# EUROPEAN PATENT SPECIFICATION

(11) **EP 0 441 421 B1**
(45) Date of publication and mention of the grant of the patent: **05.04.1995**
(21) Application number: 91200072.6
(22) Date of filing: 16.01.1991
(51) Int. Cl.: D06M 15/423, D06M 15/643

(54) **Treatment of wool**
Behandlung von Wolle
Traitement de la laine

(30) Priority: 07.02.1990 GB 9002680
(43) Date of publication of application: 14.08.1991
(73) Proprietor: BIP CHEMICALS LIMITED, Manchester M3 2NL (GB)
(72) Inventor: Heywood, Derek Wallwork, Cheadle Hulme, Cheshire (GB)
(74) Representative: Hadfield, Robert Franklin

(56) References cited:
- EP-A- 0 080 272
- GB-A- 2 217 741

## Description

This invention relates to the treatment of wool, and is particularly concerned with a process for improving its resistance to shrinkage.

A process very widely used for this purpose entails subjecting the wool to an oxidation treatment, usually a chlorination, as with free chlorine or a hypochlorite or dichloroisocyanurate salt; removing unreacted (and potentially very damaging) oxidising agent from the wool fibres, as by passage through a reducing medium such as sodium sulphite solution, followed by a water rinse; and then treating the wool with a synthetic resin to impart a resistance to shrinkage which supplements that given by the oxidation treatment. Usually thereafter, but sometimes simultaneously with the resin treatment, the wool is treated with a softening agent to soften the harsh handle which it would otherwise have as a result of the resin treatment; and in due course the treated wool is dried evenly at a moderate raised temperature to ensure that adequate curing of the resin has taken place.

The process just outlined can be applied to the treatment of wool tops (ie wool fibre before it is spun) as well as to the treatment of yarn and of woollen piece goods and garments.

Probably the resins most used in the process are those obtained by reaction of epichlorhydrin (a compound having a reactive epoxy group attached to the radical -CH₂C1) with a polyamide whose repeating unit contains basic -NH- or -NH₂ groups, as distinct from the non-basic -NH- groups of the amide linkage -CO.NH-. Such a resin is for example that obtained by the reaction of epichlorhydrin with the condensation product of a polyalkylene amine, eg diethylene triamine (H₂NCH₂CH₂NHCH₂CH₂NH₂) and adipic acid (HO₂C.CH₂CH₂CH₂CH₂CO₂H). Not all such resin is exhausted onto the wool from whatever medium the epichlorhydrin resin is applied, and there is now strong evidence that the resin-containing aqueous effluent from the proceed is harmful because of the presence in it of chlorine covalently bound to carbon, as in the -CH₂Cl group.

We have found that a treated wool product can be obtained with properties just as good as those that result when an epichlorhydrin resin is employed, by using a colloidal melamine resin as the resin to impart resistance to shrinkage. Colloidal melamine resins are used in the treatment of paper to improve its wet strength, and are obtained by dissolving a partially condensed melamine formaldehyde resin in an acid such as hydrochloric, formic, acetic or lactic acid under controlled conditions, and further diluting with water. The solution becomes infinitely miscible with water, and on ageing develops a bluish haze. The solution contains positively charged colloidal particles of the melamine resin. Such resins have also been used, in conjunction with a non-ionic silicone elastomer, in the treatment of silk, to improve crease resistance and stability to washing, as disclosed in GB-A-2217741-A.

According to the invention, there is provided a process for the treatment of wool to improve its resistance to shrinkage, by subjecting it first to an oxidation treatment and then to a colloidal melamine resin treatment to supplement the shrink resistance imparted by the oxidation treatment, the resin treatment being accompanied or followed by treatment with a softening agent to soften the harsh handle associated with use of the resin, in which process the softening agent employed is a silicone polymer.

Preferably, the silicone polymer is dispersed in the colloidal melamine resin,ie in the aqueous phase which constitutes the dispersion medium of that system.

There is described in EP-A-80272 a process for the shrink-resist treatment of wool, by
a chlorinating the wool with an acidified hypochlorite
b removing excess chlorinating agent from the wool
c applying to the acidified wool an acid colloid solution of a methylol melamine resin, which solution may contain a suitable softening agent, such as for example those of the polyethylene type.

EP-A-80272 is not, however, concerned to avoid effluent problems arising from the presence of -CH₂Cl or like groups in the resin conventionally used for wool treatment; nor does it mention the use of a silicone polymer as softening agent, a use which we have found has the advantage over polyethylene softeners of producing in the wool better stabilisation against shrinkage and better non-felting properties during washing.

The silicone polymer employed as softening agent may be cationic, but is preferably non-ionic. In general the silicone polymer used shows no chemical reactivity towards the colloidal melamine resin.

The melamine resin employed is preferably one which has at least two -CH₂OR groups per melamine nucleus, where R = H or is an alkyl group containing from one to four carbon atoms.

The invention is further illustrated by the following Examples.

### Example 1

An acidic melamine resin solution was produced by mixing the following ingredients in the following proportions by weight.

| | |
|---|---|
| Aqueous solution (80% reactive solids; pH at 1:1 H₂O dilution=8.5) of partially condensed melamine formaldehyde resin available as BEETLE® 336 | 10kg |
| Concentrated hydrochloric acid (specific gravity=1.16) | 1kg |
| Water at 40° C | 36kg |

The mixture was allowed to stand for 2 hours to develop colloidal properties, and was then diluted with an equal volume of water to give a colloidal melamine resin having a shelf life of more than 6 months.

The diluted composition (1 part by weight) was further diluted with water (4 parts) and to this mixture was added an aqueous emulsion of a non-ionic polydimethylsiloxane (0.5 parts by weight; silicone content 35% by weight). (The silicone release agent sold by Basildon Chemicals under the designation BC330 is very suitable.)

The mixed melamine resin/silicone polymer composition was then applied, from a bath adjusted with acetic acid to pH 5-6, to knitted wool garments which had been conventionally chlorinated with a dichloroisocyanurate salt, treated with antichlor, and rinsed.The bath temperature was slowly raised from ambient to 40° C during 10 minutes, and held at that temperature for a further 10 minutes to exhaust the melamine resin and silicone polymer onto the wool. Weight gain was about 1.5% by dry weight of the wool.The material was then removed from the bath, hydroextracted and tumble-dried at 60-80° C.

### Example 2

For the treatment of wool tops the procedure of Example 1 was modified as follows.

The mixed melamine resin/silicone polymer was applied in the 4th bowl of a conventional 5-bowl unit to deposit about 1.5% of solid mixture onto the tops. The treated tops were then passed to the 5th bowl, in which a cationic substituted stearamide had been included as additional softener. The tops were finally dried at 70-80° C.

## Claims

1. A process for the treatment of wool to improve its resistance to shrinkage, by subjecting it first to an oxidation treatment and then to a colloidal melamine resin treatment to supplement the shrink resistance imparted by the oxidation treatment, the resin treatment being accompanied or followed by treatment with a softening agent to soften the harsh handle associated with use of the resin, characterised in that the softening agent is a silicone polymer.

2. A process according to claim 1, in which the silicone polymer is dispersed in the colloidal melamine resin.

3. A process according to claim 1 or 2, in which the silicone polymer is non-ionic.

4. A process according to claim 3, in which the silicone polymer is a polydimethylsiloxane.

5. A process according to any of claims 1 to 4, in which the melamine resin has at least two -CH₂OR groups per melamine nucleus, where R = H or C₁₋₄ alkyl.

6. A process according to any of claims 1 to 5, in which the oxidation treatment is a chlorination.

7. A process according to claim 6, in which the chlorination utilises a dichloroisocyanurate salt.

8. A process according to any of claims 1 to 7, applied to the treatment of wool tops.

9. A process according to any of claims 1 to 7, applied to the treatment of knitted wool garments.

## Patentansprüche

1. Verfahren zur Behandlung Von Wolle zur Verbesserung ihrer Schrumpffestigkeit, indem man sie zuerst einer Oxidationsbehandlung und dann einer Behandlung mit kolloidalem Melaminharz unterzieht, um die durch die Oxidationsbehandlung verliehene Schrumpffestigkeit zu ergänzen, wobei die Harzbehandlung von einer Behandlung mit einem Erweichungsmittel begleitet wird oder davon gefolgt ist, um den harten Griff weicher zu machen, der mit der Verwendung des Harzes verbunden ist, dadurch gekennzeichnet, daß als Weichmachungsmittel ein Silikonpolymeres benutzt wird.

2. Verfahren nach Anspruch 1, dadurch gekennzeichnet, daß das Silikonpolymere im kolloidalen Melaminharz verteilt bzw. dispergiert ist.

3. Verfahren nach Anspruch 1 oder 2, dadurch gekennzeichnet, daß das Silikonpolymere nicht ionisch ist.

4. Verfahren nach Anspruch 1 oder 2, dadurch gekennzeichnet, daß das Silikonpolymere ein Polydimethylsiloxan ist.

5. Verfahren nach irgendeinem der Ansprüche 1 bis 4, dadurch gekennzeichnet, daß das Melaminharz wenigstens zwei -CH₂OR-Gruppen pro Melaminkern hat, wobei R = H oder C₁₋₄-Alkyl ist.

6. Verfahren nach irgendeinem der Ansprüche 1 bis 5, dadurch gekennzeichnet, daß die Oxidationsbehandlung eine Chlorierung ist.

7. Verfahren nach Anspruch 6, dadurch gekennzeichnet, daß die Chlorierung ein Dichlorisocyanuratsalz anwendet.

8. Verfahren nach irgendeinem der Ansprüche 1 bis 7, angewandt auf die Behandlung von Wollkammzügen.

9. Verfahren nach irgendeinem der Ansprüche 1 bis 7, angewandt auf die Behandlung von gestrickter bzw. gewirkter Wollkleidung.

## Revendications

1. Un procédé de traitement de la laine pour améliorer sa résistance au rétrécissement, en lui faisant subir d'abord un traitement d'oxydation et ensuite un traitement par une résine de mélamine colloïdale pour augmenter la résistance au rétrécissement conférée par le traitement d'oxydation, le traitement par la résine étant accompagné ou suivi de traitement par un agent d'adoucissage pour adoucir le toucher rêche associé à l'utilisation de la résine, caractérisé en ce que l'agent d'adoucissage est un polymère de silicone.

2. Un procédé selon la revendication 1, dans lequel le polymère de silicone est dispersé dans la résine de mélamine colloïdale.

3. Un procédé selon la revendication 1 ou 2, dans lequel le polymère de silicone est non ionique.

4. Un procédé selon la revendication 3, dans lequel le polymère de silicone est un polydiméthylsiloxane.

5. Un procédé selon l'une quelconque des revendications 1 à 4, dans lequel la résine de mélamine a au moins deux groupements -CH₂OR par noyau de mélamine, où R = H ou un groupement alkyle en C₁₋₄

6. Un procédé selon l'une quelconque des revendications 1 à 5, dans lequel le traitement d'oxydation est une chloration.

7. Un procédé selon la revendication 6, dans lequel la chloration utilise un sel de dichloroisocyanurate.

8. Un procédé selon l'une quelconque des revendications 1 à 7, appliqué au traitement de voiles de laine.

9. Un procédé selon l'une quelconque des revendications 1 à 7, appliqué au traitement de vêtements en laine tricotés.
